

# UNITED STATES PATENT OFFICE.

REINHOLD BECKER, OF CREFELD, GERMANY.

## HIGH-SPEED TOOL-STEEL.

1,081,263.

Specification of Letters Patent.

Patented Dec. 9, 1913.

No Drawing.

Application filed December 3, 1912. Serial No. 734,796.

To all whom it may concern:

Be it known that I, REINHOLD BECKER, a subject of the German Emperor, residing at Crefeld, Germany, have invented certain new and useful Improved High-Speed Tool-Steel, of which the following is a specification.

This invention relates to the production of a high speed tool steel which shall be easier to forge and of much greater efficiency than the best high speed tool steels hitherto known.

It has already been proposed to produce high speed tool steel from alloys of steel, tungsten, and chromium, with or without either or both of the metals vanadium and molybdenum.

According to the present invention the improved high speed tool steel consists of an alloy of steel, chromium, tungsten, and cobalt, preferably up to 15 per cent. of cobalt being employed with or without either of the metals vanadium and molybdenum.

Alloys of steel, chromium, cobalt and tungsten, or of steel, chromium, cobalt, tungsten and either vanadium or molybdenum have been found particularly suitable for the production of a high speed tool steel which is capable of being more easily worked and

is of greater efficiency than the high speed tool steels hitherto known.

In the manufacture of iron and steel it is not new *per se* to employ small quantities of cobalt, but hitherto it has only been proposed to employ cobalt in the production of weldable steel containing a high percentage of carbon. It is believed to be new, however, to employ cobalt in the manufacture of high speed tool steel having a comparatively low percentage of carbon and containing the metals, tungsten and chromium.

I claim:

1. A high speed tool steel containing chromium, tungsten, and cobalt.
2. A high speed tool steel containing a low percentage of carbon, and containing chromium, tungsten and cobalt.
3. A high speed tool steel containing a low percentage of carbon, and containing chromium, tungsten, and up to 15 per cent. of cobalt.

In testimony whereof I affix my signature in presence of two witnesses.

REINHOLD BECKER.

Witnesses:

HERMAN GLISCHTER,  
MINNA RITZEL.